

## UNITED STATES PATENT OFFICE

2,288,106

## VISCOSE SPINNING SOLUTION

Elmar Profft, Berlin-Lichterfelde, Germany, assignor to North American Rayon Corporation, New York, N. Y., a corporation of Delaware

No Drawing. Application August 3, 1939, Serial No. 288,170. In Germany August 6, 1938

9 Claims. (Cl. 106—165)

This invention relates to a method for improving the physical properties of textile structures such as filaments, threads, bands, staple fibres, and the like, made of viscose.

It is an object of the invention to improve certain of the physical properties of viscose structures of this type, including the wet and dry strengths and the wet and dry elongations as well as the dye affinity thereof by introducing certain chemical agents, e. g. organic sulphur compounds into the solutions from which such artificial structures are spun and which agents are adapted to produce effects analogous to those which impart desirable characteristics to natural products such as animal hair, wool, and the like.

A further object of the invention is to provide a method which can be practised with relatively low cost materials readily obtainable on a large scale.

It is known that in organic animal products such as wool, the sulphur, especially in the keratin, plays a very special and very unique role in that it functions to a certain extent as a connective and intermeshing bridging bond between the principal valence chains of the protein molecule. The quantity of sulphur which is necessary for forming these bridging bonds is relatively small and, as a rule, amounts to 2 to 4 per cent of the wool substance per se. It seems that the sulphur in this case is at least partially present in the form of disulphide bridging bonds. It is generally assumed that such bonds contribute appreciably to the good physical properties possessed by organic animal products, such as wool, etc.

In accordance with the present invention it has been found that it is also possible to produce an analogous effect in the case of artificial products such as viscose and hence to improve the physical properties of artificial silk, staple fibres and the like made therefrom, by adding certain sulphur-containing compounds to the viscose. More specifically, for example, organic compounds of a disulphide-like nature are added to the viscose and the viscose thus charged with sulphur compounds is spun into artificial threads, bands, staple fibres, and the like. By this means it is possible very appreciably to improve the properties of the structures spun or otherwise obtained therefrom compared to those which are spun without the addition of such sulphur-containing compounds. The dry strength as well as the wet strength thereof is appreciably increased, whereas the elongation values thereof are not only not noticeably impaired but under proper conditions are actually improved. Furthermore, the dye af-

finity of the finished product, as a rule, is also improved. Another feature of the invention resides in the fact that the addition of the disulphide-like substances to the viscose also leads to the result that the wetting capacity of the threads thus obtained is less than is customarily the case, i. e. they are less hydrophilic than normal regenerated cellulose.

It is probable that an explanation for the improvement in the physical properties of the artificial structures may be predicated upon the fact that a chemical reaction occurs between the disulphides and the cellulose, thus forming sulphur-containing bridging bonds between the 15 molecular chains and producing a sort of molecular intermeshing, that is, something similar to that inherent in keratin and also allegedly involved in the vulcanization of rubber.

The following have been found to be suitable 20 disulphide-like substances for the aforesaid purpose: higher aliphatic or cyclo-aliphatic disulphides, chlorinated higher aliphatic or cyclo-aliphatic disulphides which, for example, have taken on one mol of chlorine; and higher aliphatic or cyclo-aliphatic tetrasulphides, polysulphides, and the like. Such organic sulphur compounds are obtained, for example, by oxidation of the corresponding mercaptans and thioglycols. Exceptionally good results have been obtained 25 with mixtures of substances of the type indicated, these being derived from petroleum (or the fractions thereof which boil above 120°) and secured by the roundabout method of first producing the halogenation products and then the corresponding 30 mercaptans as set forth in my co-pending application Ser. No. 189,275, now U. S. Patent No. 2,231,594 of February 11, 1941, entitled "Process for producing improving products for pelts, furs, hairs, and textiles of all kinds," these substances 35 furthermore being well suited for the process due to their exceptional cheapness and availability in adequate quantities. It is not necessary to purify or separate these substances or mixtures, which consist, as they do, of innumerable chemical compounds of the most varied nature and of disulphide-like character, but on the contrary, the technical (crude) mixtures may even be used 40 with advantage per se directly as produced. Such substances are preferably added to the viscose in quantities amounting to about 5 to 15 per cent of the cellulose content of the viscose.

## Example I

About 1.44 kg. of a mixture of disulphides which have taken on about  $\frac{1}{2}$  mol. of chlorine

and which are obtained from petroleum indirectly by way of its chlorination products and by way of the mercaptans are intimately mixed with about 200 kg. of viscose possessing a cellulose content of about 7.2 per cent, the treated viscose being then spun into artificial silk in an acid bath containing zinc sulphate or other conventional spin baths. The physical properties of the artificial silk so obtained are better than those of artificial silk spun from viscose to which the disulphide or disulphide mixture has not been added, as shown by the following results:

|                | Strength |       | Elongation |         |
|----------------|----------|-------|------------|---------|
|                | Dry      | Wet   | Dry        | Wet     |
|                | Grams    | Grams | Percent    | Percent |
| Treated.....   | 204      | 105   | 22.1       | 38.4    |
| Untreated..... | 174      | 78    | 20.9       | 29.4    |

*Example II*

A conventional viscose solution containing about 7.2% of cellulose is spun at a maturity of about 9.5 into a spin bath containing about 250 g. of sodium sulphate, 120 g. of sulphuric acid and about 25 g. of zinc sulphate per liter of water at a speed of about 42 meters per minute and collected in a centrifugal pot revolving about 2175 times per minute. The following table clearly depicts the advantageous results obtained:

| Disulphide                                                        | Amount of disulphide (based on cellulose content) | Strength per 100 denier |       | Elongation per 100 denier |         |
|-------------------------------------------------------------------|---------------------------------------------------|-------------------------|-------|---------------------------|---------|
|                                                                   |                                                   | Dry                     | Wet   | Dry                       | Wet     |
| I. Petroleum disulphides containing about 1, mol of chlorine..... | Percent                                           | Grams                   | Grams | Percent                   | Percent |
| Petroleum disulphides.....                                        | 10                                                | 205                     | 94    | 26.4                      | 39.5    |
| Without addition of disulphides.....                              | 10                                                | 202                     | 95    | 21.1                      | 35.6    |
| II. Petroleum disulphides treated with nitric acid.....           | 0                                                 | 174                     | 78    | 20.9                      | 29.4    |
| Petroleum-bis-disulphides containing 2 S <sub>2</sub> groups..... | 10.3                                              | 181                     | 92    | 19.2                      | 28.7    |
| Without addition of disulphides.....                              | 10.3                                              | 173                     | 89    | 23.5                      | 35.8    |
|                                                                   | 0                                                 | 160                     | 85    | 18.0                      | 26.3    |

It is also to be noted that the petroleum disulphides cause a more rapid maturing of viscose solutions.

I wish to emphasize that any organic disulphide may be used in my novel process provided it is capable of chemically reacting with regenerated cellulose. Modifications of my invention will readily be recognized by those skilled in the art and I desire to include all modifications coming within the scope of the appended claims.

I claim:

1. A spinning solution for the manufacture of artificial silk comprising a viscose solution and a disulphide derived from a petroleum fraction having a boiling point above 120° C., said disulphide forming connective and intermeshing bridging bonds between the principal valence chains of the cellulose contained in said viscose solution.

2. A spinning solution for the manufacture of artificial silk comprising a viscose solution and above 120° C., said disulphide forming connective from a petroleum fraction having a boiling point about 120° C., said disulphide forming connective and intermeshing bridging bonds between the principal valence chains of the cellulose contained in said viscose solution, and said percentage being based upon the cellulose content of said viscose solution, said percentage being based upon the cellulose content of said viscose solution.

15 3. A spinning solution for the manufacture of artificial silk comprising a viscose solution and a disulphide derived from a halogenated petroleum fraction having a boiling point above 120° C., said disulphide forming connective and intermeshing bridging bonds between the principal valence chains of the cellulose contained in said viscose solution.

20 4. A spinning solution for the manufacture of artificial silk comprising a viscose solution and a disulphide derived from a chlorinated petroleum fraction having a boiling point above 120° C., said disulphide forming connective and intermeshing bridging bonds between the principal valence chains of the cellulose contained in said viscose solution.

25 5. A spinning solution for the manufacture of artificial silk comprising a viscose solution and about 5 to 15% by weight of a disulphide derived from a halogenated petroleum fraction having a boiling point above 120° C., said disulphide forming connective and intermeshing bridging bonds between the principal valence chains of the cellulose contained in said viscose solution, and said percentage being based upon the cellulose content of said viscose solution.

30 6. A spinning solution for the manufacture of artificial silk comprising a viscose solution and about 5 to 15% by weight of a disulphide derived from a chlorinated petroleum fraction having a boiling point above 120° C., said disulphide forming connective and intermeshing bridging bonds between the principal valence chains of the cellulose contained in said viscose solution, and said percentage being based upon the cellulose content of said viscose solution.

35 7. Regenerated cellulose containing a disulphide derived from a petroleum fraction having a boiling point above 120° C., said disulphide forming connective and intermeshing bridging bonds between the principal valence chains of said cellulose.

40 8. Regenerated cellulose containing a disulphide derived from a halogenated petroleum fraction having a boiling point above 120° C., said disulphide forming connective and intermeshing bridging bonds between the principal valence chains of said cellulose.

45 9. Regenerated cellulose containing a disulphide derived from a chlorinated petroleum fraction having a boiling point above 120° C., said disulphide forming connective and intermeshing bridging bonds between the principal valence chains of said cellulose.

50 60 65 ELMAR PROFFT.

CERTIFICATE OF CORRECTION.

Patent No. 2,288,106.

June 30, 1942.

ELMAR PROFFT.

It is hereby certified that error appears in the printed specification of the above numbered patent requiring correction as follows: Page 2, second column, line 3, claim 2, for "above 120° C., said disulphide forming connective" read --about 5 to 15% by weight of a disulphide derived--; line 5, same claim, for "about" read --above--; and line 10, same claim 2, strike out the comma after "solution"; and that the said Letters Patent should be read with this correction therein that the same may conform to the record of the case in the Patent Office.

Signed and sealed this 1st day of September, A. D. 1942.

(Seal)

Henry Van Arsdale,  
Acting Commissioner of Patents.